

M. UNGER.

METHOD OF PREPARING FURNACE LININGS,

APPLICATION FILED OCT. 13, 1920.

1,429,909.

Patented Sept. 19, 1922.

Fig. 1.



Fig. 2.



Fig. 3.



Inventor:  
Magnus Unger,  
by *Albert G. Davis*  
His Attorney.

## UNITED STATES PATENT OFFICE.

MAGNUS UNGER, OF PITTSFIELD, MASSACHUSETTS, ASSIGNOR TO GENERAL ELECTRIC COMPANY, A CORPORATION OF NEW YORK.

## METHOD OF PREPARING FURNACE LININGS.

Application filed October 13, 1920. Serial No. 416,670.

To all whom it may concern:

Be it known that I, MAGNUS UNGER, a citizen of the United States, residing at Pittsfield, county of Berkshire, State of Massachusetts, have invented certain new and useful Improvements in Methods of Preparing Furnace Linings, of which the following is a specification.

The present invention relates to electric induction furnaces. One of the objects of my invention is to render the lining more durable and to facilitate the curing of the lining prior to the operation of the furnace. The object is also to facilitate melting down the starting ring or initial charge.

The induction furnace linings commonly are made by ramming refractory material, together with suitable binder, about a form or templet and then curing the green lining thus made by subjecting it to heat from a ring of metal placed in the furnace crucible, constituting a secondary winding of the furnace.

It has been suggested to build the furnace lining about a templet of metal having a contour corresponding to the desired shape of the furnace chamber and then to utilize the templet for baking out the furnace lining without removing the templet and finally melting down the templet. Due to the differences in thermal expansion coefficients of metals and of the refractory materials used for furnace linings the lining is very apt to be cracked when the templet is heated. Furthermore in attempting to melt down the templet by inducing a current therein, the pinch effect is likely to prematurely rupture the metal and break the circuit before the lining is fully baked out. The result of such a break in the circuit is a very difficult and time consuming matter.

In accordance with my present invention the green furnace lining is shaped in any desired way and then baked out by a composite heater conforming, in a general way, to the contour of the lining but spaced away therefrom and consisting of rings of metal of different melting points. The pinch force is not likely to rupture the metal circuit unless the metal is near or above its melting point. In case the circuit of metal having the lowest melting point should be ruptured there will be sufficient heat generated in the circuit having the higher melting point to

cause the metal in the ruptured circuit to melt.

In the accompanying drawing, Fig. 1 is a vertical section through an induction furnace illustrating a composite heater in the first stage of the baking out of a furnace crucible; Fig. 2 is a section of the furnace crucible showing the second stage of a preparation of the crucible; and Fig. 3 is a sectional view illustrating the third and final stage.

The furnace crucible shown in Fig. 1 comprises a wall of fire-brick surrounding a mass of refractory material 2 consisting of highly refractory material suitable for furnace lining. For example, this inner layer 70 tube may consist of a mixture of magnesia which has been subjected to fusion and of magnesia which has been highly sintered short of fusion. These two materials in a comminuted state together with a suitable 75 binder, as for example, tar or magnesium chloride or sulphate, are rammed into position about a templet of desired form. Preferably, a spacer is placed between the wall 1 and the lining 2 and when the lining has 80 been rammed into position this spacer is removed and the space filled with some suitable powdered or flocculent refractory material as indicated at 3. Powdered magnesia in the sintered state may be used. This loose 85 layer permits the lining layer 2 to expand when heated.

When the inner core or templet has been removed leaving an annular chamber 4, a plurality of starting rings 5 and 6 are placed 90 within the chamber 4, these rings being shaped so as to conform in a general way with the configuration of the lining 2 but leaving a space between the side walls of the chamber 4 and the sides of the rings particularly adjacent the upper ring. These rings 5 and 6 consist of metals melting at different temperatures. When the furnace is to be used for production of steel, I prefer to use rings of ferrous metals having different 100 melting points, for example, the upper ring 5 may consist of cast steel and the lower ring 6 of cast iron. In the same manner rings of steel of different melting points may be used.

When the furnace lining has been shaped and the rings have been placed in position, the temperature of the rings is gradually

raised by induction in the usual manner (the magnetic core and the primary winding of the furnace have been omitted for the sake of simplicity). For example, when curing 5 a lining consisting of magnesia and tar as above described, the temperature of the rings 5 and 6 is gradually increased from room temperature to about 1100° C. through a period of about 18 hours, thereby volatilizing 10 and carbonizing the tar binder and otherwise curing the lining 2. At a temperature of 1100° C. the cast iron ring 6 will melt allowing the ring 5 to float in the molten cast iron as indicated in Fig. 2. 15 During the period that the steel ring 5 remains unfused and floating upon the molten mass 7, the molten mass in the bottom of the crucible is not likely to be open-circuited by the pinch effect. In case there 20 should be a break in the upper ring the break will be closed immediately by the metal of the lower melting point.

The temperature finally is gradually increased by increasing the current in the 25 primary of the furnace so as to bring the temperature up to about 1450° C. during the period of about 4 hours. At this temperature the steel ring 5 will also melt and mix with the cast iron producing a molten charge 30 as indicated at 8 in Fig. 3. The temperature is now raised over an additional period of about 2 hours to about 1550° C. The furnace is then ready for use.

What I claim as new and desire to secure 35 by Letters Patent of the United States, is:

1. The method of starting an induction furnace which consists in placing within the heating space of said furnace a plurality of closed conductors respectively melting at different temperatures, and inducing a heating current therein of sufficient power to successively melt said conductors.

2. The method of starting an induction furnace which consists in placing within the 45 heating space of said furnace a cast-iron ring, and a larger ring of cast steel, melting said cast-iron ring by induced current and thereupon melting said cast steel ring.

3. The method of preparing for use a 50 green lining for an induction furnace which consists in subjecting said lining to the heat-

ing effect of a compound heater having a surface contour conforming substantially to the contour of said lining but spaced away therefrom, said body consisting in larger 55 part of a ring of steel and in lesser part of a ring of cast iron, inducing a current in said heater sufficient to bake out said lining, and finally successively melting the parts of said heater.

4. The method of curing the linings of electric induction furnaces which consists in subjecting said linings to the heating effect of a composite conductive body consisting of materials melting at different temperature having a surface contour conforming substantially to the contour of said lining but spaced away therefrom when expanded by heat and finally melting successively the constituents of said body.

5. The method of preparing linings for electric induction furnaces which consists in shaping a lining material around a templet of desired form, removing said templet when said material is in a desired position, 75 placing in the space within said lining a plurality of metal rings proportioned to be spaced away from the side walls of the lining when heated, inducing a heating current in said body to bake said lining and finally melting said rings successively to completely consolidate said lining.

6. The method of starting an induction furnace with a green lining which consists in charging said furnace with rings of 85 ferrous metal, having different melting points, heating said rings by induction to cure said lining and thereupon melting said rings by induction.

7. The method of curing the linings of a 90 furnace chamber which consists in subjecting said lining to the heating effect of a current induced in a plurality of metal rings consisting of materials melting at different temperatures above the temperature range 95 in which volatilizable constituents of said lining are eliminated and finally by successive increases of temperature melting said rings in said chamber.

In witness whereof, I have hereunto set 100 my hand this eighth day of October, 1920.

MAGNUS UNGER.